

Feb. 9, 1937.

G. F. WEATON ET AL

2,070,101

CONDENSATION OF METALLIC VAPORS

Filed May 5, 1936



Inventors:

George F. Weaton  
Herard K. Najarian  
Potter, Pierce & Scheffler Attorneys.

## UNITED STATES PATENT OFFICE

2,070,101

## CONDENSATION OF METALLIC VAPORS

George F. Weaton and Herand K. Najarian,  
Beaver, Pa., assignors to St. Joseph Lead Com-  
pany, New York, N. Y., a corporation of New  
York

Application May 5, 1936, Serial No. 78,060  
In Great Britain February 11, 1935

18 Claims. (Cl. 266—19)

This invention relates to an improved method and apparatus for the condensation of metallic vapors of the volatile metals, particularly zinc, by passing the metallic vapor into an enclosed mass of molten metal wherein it is subject to such conditions that condensation of the vapor therein is practically complete.

The invention makes possible continuous and highly efficient condensation of zinc vapor with avoidance of the production of any material amount of blue powder.

In accordance with the preferred practice of the invention, the zinc vapor and accompanying gases, from which air is excluded, are conducted from the furnace through an insulated conduit to an insulated entrance chamber, thus maintaining the vapor and gases at a temperature above the condensation point of the vapor. From the entrance chamber, which is contiguous to one end of a receptacle enclosing a mass of molten zinc, the vapor and gases are introduced into said mass at a substantial distance below its upper exposed surface which is at the opposite end of the receptacle.

At the other end of the receptacle is an exit chamber into which the uncondensed gases escape after passing through the mass of molten metal. A suction is applied to draw off these gases, which is sufficiently strong to raise and maintain the level of the upper exposed surface of the molten metal at the necessary substantial height above the level of its lower exposed surface and to depress and maintain said lower surface at a level that permits the vapor and gases to enter the mass of molten metal just above said lower exposed surface.

The vapor and gases are maintained submerged in said mass by the inclined enclosing roof of said receptacle and travel upwards in an inclined path through the circumferentially confined mass of molten metal. Baffles in the receptacle impede the flow of the vapor and gases in the molten metal and increase the turbulence caused by vapor condensation. Thus the molten metal is violently agitated and the vapor and gases are dispersed and broken up into bubbles which are intimately mixed with the molten metal. The flow of the vapor and gases through the relatively cool molten metal is retarded therein for a sufficient time to permit complete condensation of substantial volumes of vapor before it can escape from the molten metal. As the vapor in the molten metal comes in contact only with such metal and with surfaces actively wiped thereby, the condensation of zinc vapor is

accomplished substantially without the production of blue powder.

The invention, while particularly described with reference to zinc, may be applied to the condensation of other volatile metals such as mercury, cadmium, magnesium and tin.

The invention will be more particularly described with reference to the accompanying drawing showing the preferred form of apparatus in which:

Fig. 1 is a schematic representation, with portions broken away, of equipment embodying the invention; and

Fig. 2 is a vertical section on line 2—2 of the condenser illustrated in Fig. 1.

The vapors and the gases are conducted from the furnace, not shown, where they are generated, through a heat insulated conduit 21, into an entrance chamber 2 which is likewise heat insulated.

A condensing receptacle 1, which may be of any desired shape, but is preferably tubular and ovoid in cross-section (as shown in Fig. 2), although not necessarily so, connects the lower end of the entrance chamber 2 with an exit chamber 25

3. The roof portion of this receptacle is advantageously inclined at an angle of from 45° to 75°, preferably from 55° to 65°, from the vertical. A pipe leads from the exit chamber 3 to an exhaust pump 4 which pumps the gases, escaping from the exposed upper surface of the liquid mass, from the exit chamber into a gas holder 14. This pump is sufficiently powerful to maintain in the exit chamber a reduction in the gas pressure below atmospheric equivalent to at least 20 six inches of mercury and thus serves not only to remove by suction the escaping gases, but also to create and maintain the substantial difference in level between the exposed surfaces in said exit and entrance chambers, respectively, as is 40 necessary for successful operation. The elongated or tubular condensing receptacle 1 is preferably constructed with a metal casing 17 having a refractory lining 18. It is advantageously provided internally with baffles 5 depending from 45 its roof and with surge baffles 6 extending across the receptacle. To regulate the temperature of the molten metal, which is raised by the vapor condensation, the exterior of the condensing receptacle 1 may be cooled by liquid sprayed from the pipe 15 and collected in the trough 15'. The molten metal may be tapped off through any suitable outlet communicating with the molten metal in the condensing chamber, in inlet chamber 2, or in outlet chamber 3, but in the apparatus 50

10

15

20

25

30

35

40

45

50

55

shown we provide an automatic discharge. At or near the connection of the upper end of the receptacle 1 to the exit chamber 3 is a horizontal outlet having a downwardly depending curtain 7 and a dam 8 that leads to a barometric leg 9. This leg leads to a forehearth 10 for holding the molten metal which may be withdrawn therefrom into molds. Above chamber 3 there may be a gas washer 12 provided with sprays 11 draining into sump 13 through pipes 19 and 20.

To initiate the operation, the receptacle 1 is first provided with a suitable amount of molten metal. Reduced gas pressure in the exit chamber 15 is created and maintained by the exhaust pump. This lifts the upper exposed surface of the molten metal towards or above the upper level 1a and depresses the exposed surface of the liquid at the lower end of the entrance chamber 20 2 to the level 1b, so that the level 1b is below the lower end 16 of the inclined roof portion of the receptacle and is a substantial vertical distance below the level 1a. By "substantial" we 25 mean that this distance is sufficient, under the conditions present, to provide a path for the flow of the vapor in the liquid mass that is long enough to allow time for the condensation in that mass of large volumes of vapor. The vertical height from 1b to 1a is, in the case of the 30 preferred apparatus herein described, when used for the condensation of zinc, at least 12 inches. As the level of the lower exposed surface of the liquid 1b is below the corner 16, the vapor and gases from the furnace flow from the entrance chamber 2 under the corner 16 and into the circumferentially confined mass of molten metal 35 in the receptacle 1. Said receptacle, for its length from just beyond the corner 16 to the upper exposed surface 1a, is in normal operation 40 filled throughout its transverse cross-section with the mass of molten metal through which the vapor forces its passage until condensed therein.

The inclination of the roof of the receptacle from the vertical, along and against which roof 45 the vapor and the gases try to flow, retards their flow through the molten metal by providing an inclined path for such flow, which is preferably at least twice as long as the vertical distance between the corner 16 and the level of the upper 50 exposed surface 1a of the molten metal. The baffles 5 and 6, submerged in the liquid mass in receptacle, serve to retard further that flow and also to agitate the vapor and gases in the molten metal, the baffles 6 being particularly effective 55 in preventing objectionable surging of such metal.

The vapor and gases are thus agitated, broken up and subdivided into bubbles and dispersed through the molten metal and, by providing a 60 sufficiently long path for their travel within the liquid and retarding their flow therein, sufficient time is provided for the complete condensation of large volumes of metallic vapor. To maintain the liquid metal at substantially the desired constant 65 temperature, it is cooled by any suitable means, as, for example, by spraying the outside of the condenser receptacle by water sprays 15. Thus conditions for the most efficient condensation of the vapor in the liquid mass are realized.

70 As the volume of liquid metal increases, due to the condensation of the metallic vapor, the surplus may be tapped off. As shown, such surplus flows over the dam 8 through the barometric leg 9 into the forehearth 10. The uncondensed 75 gases drawn from the exit chamber 2 may be

collected in gas holder 14 after being washed by the sprays 11. The solids may be collected in receptacle 13.

In the process of our invention, above set forth, the zinc vapor has little or no opportunity to form blue powder. Before it enters the mass of molten metal it is maintained at a temperature above that of its condensation. When in said liquid mass the vapor comes in contact only with molten metal and with surfaces of the receptacle which are submerged in and energetically wiped by the agitated molten metal. As these surfaces are the only surfaces with which the vapor comes in contact, that are below the temperature of its condensation, 15 the formation of blue powder is practically eliminated. If perchance there should be some particles of blue powder in the mass of molten metal, the heat and agitation of the molten zinc tend to amalgamate these particles with the molten 20 metal and thus rid the mass of molten metal of them.

This application is a continuation-in-part of applications Serial No. 714,730 and Serial No. 714,731, filed March 8, 1934.

25 We claim:

1. The method of condensing zinc vapor which comprises providing a mass of molten zinc circumferentially confined except at opposite ends thereof, conducting gases and zinc vapor from 30 a furnace to the exposed surface of said mass at one end thereof while maintaining the temperature of said vapor above the condensation point thereof, drawing off the gases from a space above the exposed surface of said mass at the opposite end thereof by suction equal to at least 6 inches of mercury, thereby raising the liquid zinc at said latter end and lowering it at the former end so that the level of the upper exposed surface of the liquid is at least 12 inches higher vertically 35 than the level of the lower exposed surface of the liquid and said lower exposed surface is brought to a level that permits said gases and vapor to flow into said mass of liquid at least 12 inches below its upper exposed surface, conducting said gases and 40 vapor in said mass in an inclined upward direction, impeding the flow of said gases and vapor in said mass thereby agitating and breaking up the same into bubbles 45 and retarding their flow, contacting said bubbles 50 in said mass only with the molten metal or with surfaces wiped by said metal, retaining said vapor in said mass for sufficient time to condense substantially all of it, delivering the uncondensed gases to the space above the upper 55 exposed surface of said mass, regulating the temperature of said mass of liquid by cooling it, and drawing off the accumulated molten metal.

2. The method of condensing zinc vapor which comprises providing a mass of molten 60 zinc circumferentially confined except at opposite ends thereof, conducting gases and zinc vapor from a furnace to the exposed surface of said mass at one end thereof, drawing off the gases from a space above the exposed surface 65 of said mass at the opposite end thereof by a suction powerful enough to raise the exposed surface of liquid zinc at one end at least 12 inches higher vertically than the level of the other exposed surface of the liquid and to depress said lower exposed surface to a level that permits said gases and vapor to flow into said mass of liquid at least 12 inches below its upper exposed surface, conducting said gases and 70 vapor in said mass in an inclined upward di- 75

rection, impeding the flow of said gases and vapor in said mass thereby agitating and breaking up the same into bubbles and retarding their flow, contacting said bubbles in said mass only with the molten metal or with surfaces wiped by said metal, retaining said vapor in said mass for sufficient time to condense substantially all of it, and delivering the uncondensed gases to the space above the upper exposed surface of said mass.

3. The method of condensing zinc vapor which comprises providing a mass of molten zinc circumferentially confined except at opposite ends thereof, conducting gases and zinc vapor from a furnace to the exposed surface of said mass at one end thereof, drawing off the gases from a space above the exposed surface of said mass at the opposite end thereof by suction, thereby raising the level of the exposed surface of the liquid zinc at said latter end and depressing it at the former end so that the lower exposed surface is brought to a level that permits said gases and vapor to flow into said body of liquid at least 12 inches below its upper exposed surface, and retaining said vapor in said mass for sufficient time to condense substantially all of it.

4. The method of condensing zinc vapor which comprises providing a mass of molten zinc circumferentially confined except at opposite ends thereof, conducting gases and zinc vapor from a furnace to the exposed surface of said mass at one end thereof, drawing off the gases from a space above the exposed surface of said mass at the opposite end thereof by suction, thereby raising the level of the exposed surface of the liquid zinc at said latter end and depressing it at the former end so that said lower exposed surface is brought to a level that permits said gases and vapor to flow into said mass of liquid at least 12 inches below its upper exposed surface, conducting said gases and vapor in said mass in an inclined upward direction, and retaining said vapor in said mass for sufficient time to condense substantially all of it.

5. The method of condensing zinc vapor which comprises providing a mass of molten zinc circumferentially confined except at opposite ends thereof, conducting gases and zinc vapor from a furnace to the exposed surface of said mass at one end thereof, drawing off the gases from a space above the exposed surface of said mass at the opposite end thereof by suction, thereby raising the liquid zinc at said latter end and lowering it at the former end so that the level of the upper surface of the liquid is substantially higher vertically than the level of the lower surface of the liquid and said lower surface is brought to a level that permits said gases and vapor to flow into said mass of liquid substantially below its upper surface, partially obstructing the flow of said gases and vapor in said mass thereby agitating and breaking up the same into bubbles and retarding their flow, contacting said bubbles in said mass only with the molten metal or with surfaces wiped by said metal, retaining said vapor in said mass for sufficient time to condense substantially all of it, delivering the uncondensed gases to the space above the upper surface of said mass, and drawing off the accumulated molten metal.

6. The method of condensing zinc vapor which comprises providing a mass of molten zinc circumferentially confined except at opposite ends thereof, conducting gases and zinc vapor from a furnace to the exposed surface of said

mass at one end thereof, drawing off the gases from a space above the exposed surface of said mass at the opposite end thereof by suction, thereby raising the liquid zinc at said latter end and lowering it at the former end so that the level of the upper surface of the liquid is substantially higher vertically than the level of the lower surface of the liquid and said lower surface is brought to a level that permits said gases and vapor to flow into said mass of liquid substantially below its upper surface, conducting said gases and vapor in said mass in an inclined upward direction, partially obstructing the flow of said gases and vapor in said mass thereby agitating and breaking up the same into bubbles and retarding their flow, contacting said bubbles in said mass only with the molten metal or with surfaces wiped by said metal, retaining said vapor in said mass for sufficient time to condense substantially all of it, delivering the uncondensed gases to the space above the upper surface of said mass, regulating the temperature of said mass of liquid by cooling it, and drawing off the accumulated molten metal.

7. Apparatus for the condensation of metallic vapors such as zinc or the like comprising, in combination, a heat insulated entrance chamber connected to a source of gases and said vapors, an exit chamber, a receptacle having its respective ends connected to said chambers and normally filled with molten metal for a substantial portion of its length throughout its transverse cross-section, a suction producing device to draw off gases from said exit chamber and to lift the exposed upper surface of said metal substantially above its exposed lower surface, an enclosing roof portion to said receptacle in contact with and confining said molten metal intermediate said chambers, and baffles submerged in said receptacle to impede and retard the flow of gases and vapors therein, whereby said vapors are condensed in said molten metal and the uncondensed gases are delivered to said exit chamber.

8. Apparatus for the condensation of metallic vapors such as zinc or the like comprising, in combination, a heat insulated entrance chamber connected to a source of gases and said vapors, an exit chamber, a receptacle having its respective ends connected to said chambers and normally filled with molten metal for a substantial portion of its length throughout its transverse cross-section, a suction producing device to draw off gases from said exit chamber and to lift the exposed upper surface of said metal substantially above its exposed lower surface, an inclined enclosing roof portion to said receptacle in contact with and confining said molten metal intermediate said chambers and inclined between 45° and 75° from the vertical, and baffles in said receptacle to retard the flow of gases and vapors along said roof portion, whereby said vapors are condensed in said molten metal and the uncondensed gases are delivered to said exit chamber.

9. Apparatus for the condensation of metallic vapors such as zinc or the like comprising, in combination, a heat insulated entrance chamber connected to a source of gases and said vapors, an exit chamber, a receptacle having its respective ends connected to said chambers and normally filled with molten metal for a substantial portion of its length throughout its transverse cross-section, a suction producing device to draw off gases from said exit chamber and to lift the

exposed upper surface of said metal substantially above its exposed lower surface, an inclined enclosing roof portion to said receptacle in contact with and confining said molten metal intermediate said chambers and inclined between 55° and 65° from the vertical, and baffles in said receptacle to retard the flow of gases and vapors along said roof portion, whereby said vapors are condensed in said molten metal and the uncondensed gases 10 are delivered to said exit chamber.

10. Apparatus for the condensation of metallic vapors such as zinc or the like comprising, in combination, a heat insulated entrance chamber connected to a source of gases and said vapors, an exit chamber, a receptacle having its respective ends connected to said chambers and normally filled with molten metal for a substantial portion of its length throughout its transverse cross-section, a suction producing device to draw off gases from said exit chamber and to lift the exposed upper surface of said metal substantially above its exposed lower surface, an inclined enclosing roof portion to said receptacle in contact with and confining said molten metal intermediate said chambers and at least twice as long as the vertical distance between said exposed surfaces, submerged baffles in said receptacle to impede and retard the flow of gases and vapors along said roof portion, whereby said vapors are 20 condensed in said molten metal and the uncondensed gases are delivered to said exit chamber.

11. Apparatus for the condensation of metallic vapors such as zinc or the like comprising, in combination, a heat insulated entrance chamber connected to a source of gases and said vapors, an exit chamber, a receptacle having its respective ends connected to said chambers and normally filled with molten metal for a substantial portion of its length throughout its transverse cross-section, a suction producing device to draw off gases from said exit chamber and to lift the exposed upper surface of said metal substantially above its exposed lower surface, an inclined enclosing roof portion to said receptacle in contact with and confining said molten metal intermediate said chambers, and submerged baffles in said receptacle, to obstruct and to retard the flow of gases and vapors therein, whereby said vapors are 30 condensed in said molten metal and the uncondensed gases are delivered to said exit chamber.

12. Apparatus for the condensation of metallic vapors such as zinc or the like comprising, in combination, a heat insulated entrance chamber connected to a source of gases and said vapors, an exit chamber, a receptacle having its respective ends connected to said chambers and normally filled with molten metal for a substantial portion of its length throughout its transverse cross-section, a suction producing device to draw off gases from said exit chamber and to lift the exposed upper surface of said metal substantially above its exposed lower surface, an inclined enclosing roof portion to said receptacle in contact with and confining said molten metal intermediate said chambers to impede and retard the flow of gases and vapors along said roof portion, whereby said vapors are 40 condensed in said molten metal.

13. Apparatus for the condensation of metallic vapors such as zinc or the like comprising, in combination, a heat insulated entrance chamber connected to a source of gases and said vapors, an exit chamber, a receptacle having its respective ends connected to said chambers and normally filled with molten metal for a substantial portion 50 of its length throughout its transverse cross-section,

tion, a suction producing device to draw off gases from said exit chamber and to lift the exposed upper surface of said metal substantially above its exposed lower surface, an enclosing roof portion to said receptacle inclined between 45° and 75° from the vertical and in contact with and confining said molten metal intermediate said chambers to impede and retard the flow of gases and vapors along said roof portion, whereby said vapors are 55 condensed in said molten metal.

14. Apparatus for the condensation of metallic vapors such as zinc or the like comprising, in combination, a heat insulated entrance chamber, connected to a source of gases and said vapors, an exit chamber, a receptacle having its respective ends connected to said chambers and normally filled with molten metal for a substantial portion of its length throughout its transverse cross-section, a suction producing device to draw off gases from said exit chamber and to lift the 20 exposed upper surface of said metal substantially above its exposed lower surface, said receptacle having an enclosing roof portion in contact with and confining said molten metal intermediate said chamber, and submerged transverse baffles along the roof portion of said receptacle to obstruct and impede the flow of gases and vapors 25 therein, whereby said vapors are condensed in said molten metal.

15. Apparatus for the condensation of metallic vapors such as zinc or the like comprising, in combination, a heat insulated entrance chamber connected to a source of gases and said vapors, an exit chamber, a receptacle having its respective ends connected to said chambers and normally filled with molten metal for a substantial portion of its length throughout its transverse cross-section, said receptacle having an inclined enclosing roof portion in contact with and confining said molten metal intermediate said chambers, a suction producing device to draw off gases from said exit chamber and to lift the exposed upper surface of said metal and depress its exposed lower surface below the lower end of said roof portion, and submerged transverse baffles in said receptacle spaced from the roof portion thereof to prevent surging of the molten metal.

16. Apparatus for the condensation of metallic vapors such as zinc or the like comprising, in combination, a heat insulated entrance chamber connected to a source of gases and said vapors, an exit chamber, a receptacle having its respective ends connected to said chambers and normally filled with molten metal for a substantial portion of its length throughout its transverse cross-section, said receptacle having an inclined enclosing roof portion in contact with and confining said molten metal intermediate said chambers, and a suction producing device to draw off gases from said exit chamber and to create and maintain the exposed lower surface of said molten metal below the lower end of said roof portion, whereby said vapors are introduced into said molten metal immediately above the lower exposed surface thereof.

17. Apparatus for the condensation of metallic vapors such as zinc or the like comprising, in combination, a heat insulated entrance chamber connected to a source of gases and said vapors, an exit chamber, a receptacle having its respective ends connected to said chambers and normally filled with molten metal for a substantial portion of its length throughout its transverse cross-section, said receptacle having an inclined enclosing roof portion in contact with and con- 70

fining said molten metal intermediate said chambers and a suction producing device to draw off gases from said exit chamber and to create and maintain the exposed lower surface of said molten metal below the lower end of said roof portion, whereby said vapors are introduced into said molten metal immediately above the lower exposed surface thereof, and baffles in said receptacle to impede and retard the flow of the vapors therein.

18. A method of condensing zinc vapors which comprises passing the zinc vapors into a body of zinc in liquid form and retarding the passage of vapors through the liquid zinc so that substantially all of the zinc is condensed in contact only with the liquid zinc and with surfaces actively wiped by the liquid zinc. 5

GEORGE F. WEATON.  
HERAND K. NAJARIAN. 10